

## UNITED STATES PATENT OFFICE

2,227,149

## LUBRICATING OIL FOR DIESEL ENGINES

Eger V. Murphree, Summit, N. J., assignor to  
Standard Oil Development Company, a corpora-  
tion of Delaware

No Drawing. Application December 23, 1937,  
Serial No. 181,374

12 Claims. (Cl. 252—35)

This invention relates to lubricating oils for Diesel engines and is more particularly concerned with certain addition agents which when added to non-waxy lubricating oils greatly improve their properties.

It is known that certain metallic soaps such as aluminum stearate and aluminum naphthenate improve the properties of lubricating oils for Diesel engines particularly with respect to decreasing ring sticking and varnish forming tendencies as well as increasing oiliness. A serious objection to the use of aluminum stearate for this purpose is that it tends to settle out or gel upon standing. An objection to the use of aluminum naphthenate is that it requires a temperature of 300 to 400° F. for solution in oil, and at these temperatures color deterioration is inevitable and unavoidable.

It is desirable to use a metallic soap which has all of the desirable properties of these aluminum soaps but which does not settle out on standing and does not require temperatures for solution high enough to cause color deterioration.

It has now been found that metallic soaps of acids obtained by the oxidation of "sweater oil" form extremely stable solutions in non-waxy lubricating oils and can be completely dissolved in amounts of 0.1 to 3% in lubricating oil at temperatures between 175 and 200° F. at which no color deterioration occurs. The nature of these soaps and the method of preparing them will be fully understood from the following description:

In dewaxing an oil containing pressable wax, the wax precipitated in the process is called crude slack wax. This contains varying quantities of oil which is carried down with the wax. The crude slack wax is warmed to sweat out the oil. The sweated wax is called crude scale wax, and the oil obtained is called foots oil. The crude scale wax is subjected to another sweating operation and the oil so obtained is called "sweater oil." It is this sweater oil obtained from the sweating of crude scale wax which is used as the starting material for the preparation of the acids desired in the present process.

Sweater oil is distinguished from crude scale wax by the fact that it contains relatively much larger quantities of oil.

The "sweater oil" is oxidized with air or other gas containing free oxygen at a temperature between about 200 and 350° F. for a period of 2 to 4 hours. Various catalytic materials such as potassium permanganate, manganese stearate or soda ash may be used to promote the oxidation. The reaction product is then saponified with caustic soda preferably containing some methyl alcohol. Thereafter, the mixture is thoroughly agitated and the aqueous layer is separated from the oily layer. The aqueous layer contains the sodium soaps of the desired acids along with a small amount of unsaponifiable materials. The unsaponifiable materials are then removed either by naphtha extraction or by vaporization. Sulfuric acid is added to the sodium soaps to liberate the acids. The acids are then washed and distilled, and either a fraction of the distillate or the entire distillate and bottoms may be used for preparing the desired metallic soaps.

In preparing aluminum soaps from the acids, the alkali (sodium, for example) soap is first prepared. The alkali soap solution is then added to an aluminum sulfate solution, a slight excess of the latter being used. It will be understood that if other metallic soaps are desired, appropriate solutions of the metal salts will be used or the soaps may be prepared by direct cooking of the acids with appropriate metallic oxides or hydroxides.

The aluminum soap is washed free of inorganic salts and may then be dried or may be incorporated directly in the oil without drying, in which latter case the moisture is removed from the compounded oil by blowing with air or an inert gas.

The metallic soap is added to the oil in amounts of 0.1 to 3%. The oil is heated to a temperature between about 175 and 200° F. and the soap stirred into it.

Various other metals besides aluminum may be used, such as calcium, nickel, cobalt, magnesium, manganese, chromium, tin, zinc, etc. These soaps may be prepared as indicated above by adding the sodium soap to a solution of the metallic salt. Other methods of preparation are, of course, not precluded.

In preparing the soap, the entire acid fraction may be used or only a portion thereof. It is found that the No. 6 cut obtained by vacuum

and steam distillation at 4 mm. of mercury and boiling between about 150 and 280° C. is particularly suitable. This fraction constitutes from 50 to 65% of the entire acid product.

5 The acid numbers and saponification numbers of the total acid and No. 6 cut respectively are approximately as follows:

| 10                      | Acid No. | Saponification number |
|-------------------------|----------|-----------------------|
| Crude acid product..... | 161      | 238                   |
| No. 6 cut.....          | 175      | 239                   |

15 It is found that the soaps prepared from "sweater oil" acids are markedly different in properties from those prepared from oxidized scale wax. For example, the acid and saponification numbers compare as follows:

| 20                                       | Acid No. | Saponification number |
|------------------------------------------|----------|-----------------------|
| 25 No. 6 cut of oxidized scale wax.....  | 206      | 230                   |
| No. 6 cut of oxidized "sweater oil"..... | 175      | 240                   |

It is also found that the soaps of the No. 6 cut of oxidized scale wax as such are substantially insoluble in mineral oils whereas the soap of the 30 No. 6 cut of "sweater oil" acids are relatively much more soluble.

The following example illustrates the use of the improved soap:

35 1.7% of aluminum soap of the No. 6 cut of the distillate of acids prepared by the oxidation of "sweater oil" is added to a non-waxy naphthenic oil obtained from a Coastal crude and having a Saybolt Viscosity at 210° F. of 55 seconds and the mixture heated to about 175 to 200° F. until 40 complete solution is effected. After standing in storage for 3½ months, the oil shows no haze, gelling or other evidence of separation of the soap, but remains clear, bright and of excellent appearance.

45 This oil was tested for 250 hours operation on a Caterpillar Diesel engine and showed superior performance over blends of aluminum naphthenate or the aluminum soap of acids derived from the oxidation of crude scale wax in the 50 same oil.

In some instances, e. g. in the case of the calcium, magnesium, zinc, manganese and similar soaps, difficulties may be encountered in dissolving them in certain mineral lubricating oils. In 55 such cases, it has been found advantageous to add a solubilizing agent (about 5-100% or more of the weight of the soap added) to prevent gel formation and to overcome other effects of deficiency in solubility of the soaps. Such solubilizers may be higher free fatty acids, fatty esters, naphthenic acids or esters, aromatic fatty acids such as phenyl stearic acid or their esters, organic esters of inorganic acids or aromatic polybasic acids, high molecular weight alcohols, alcohol-esters, alcohol-ethers, ether-esters, and other similar high boiling compounds.

60 It will be understood that other addition agents besides the aluminum soaps may be added to the Diesel oils, such as oiliness agents, corrosion inhibitors, oxidation inhibitors, extreme pressure agents, thickeners, dyes, etc.

65 The use of these soaps is not restricted to any particular type of non-waxy lubricating oil but is applicable generally to all Diesel lubricating

fractions whether obtained by the distillation, cracking, hydrogenation, destructive hydrogenation or other treatment of petroleum, coals, tars, shales, lignites or fractions thereof.

70 This invention is not limited by any theories of the mechanism of the reactions nor by any details which have been given merely for purposes of illustration, but is limited only in and by the following claims in which it is intended to claim all novelty inherent in the invention. 10

I claim:

1. An improved lubricating oil composition for internal combustion engines comprising a lubricating oil containing a small amount of polyvalent metal soap of acids derived from the oxidation of "sweater oil." 15

2. An improved lubricating oil for Diesel engines comprising a non-waxy lubricating fraction containing from 0.1 to 3% of a polyvalent metal soap of acids derived from the oxidation 20 of "sweater oil."

3. An improved lubricating oil for Diesel engines comprising a non-waxy lubricating fraction of petroleum containing 0.1 to 3% of a polyvalent metal soap of acids derived from the oxidation 25 of "sweater oil."

4. Lubricating oil according to claim 3 in which the soap is prepared from a metal selected from the class consisting of aluminum, calcium, nickel, tin and magnesium. 30

5. An improved lubricating oil for Diesel engines comprising a non-waxy lubricating oil containing 0.1 to 3% of an aluminum soap of acids derived from the oxidation of "sweater oil."

6. An improved lubricating oil for Diesel engines comprising a non-waxy lubricating oil containing 0.1 to 3% of an aluminum soap of an acid fraction boiling between 150 and 280° C. at 4 mm. of mercury with steam obtained from the products of oxidation of "sweater oil." 40

7. An improved lubricating oil composition according to claim 1 in which the soap is oil soluble.

8. An improved lubricating oil composition for internal combustion engines comprising a lubricating oil containing a small amount of a polyvalent metal soap of acids derived from the oxidation of sweater oils, the solubility of said metal soap being increased by the addition of an organic solubilizer. 45

9. A composition according to claim 8 in which the organic solubilizer is a higher fatty acid. 50

10. A composition according to claim 8 in which the solubilizer is a higher alcohol.

11. A method of making an improved lubricating oil composition especially adapted for lubrication of Diesel engines, which comprises oxidizing a "sweater oil" fraction of petroleum hydrocarbons, to produce acid derivatives thereof, converting said acids into corresponding polyvalent metal soaps, and incorporating from 0.1 to 3% of such metal soap into a lubricating oil. 55

12. A method of preparing an improved lubricating oil composition for lubrication of Diesel engines which comprises subjecting a "sweater oil" fraction of petroleum hydrocarbons to oxidation with air at a temperature between about 200° and 350° F. for a period of 2-4 hours to prepare acid derivatives thereof, recovering the acids from said reaction product, converting them into corresponding aluminum soaps, and incorporating 0.1 to 3% of said aluminum soap into a non-waxy lubricating fraction of petroleum. 60